

Patented Oct. 25, 1927.

1,646,625

# UNITED STATES PATENT OFFICE.

WILLIAM MENDEL, OF BEVERLY, NEW JERSEY, ASSIGNOR TO SAMUEL A. NEIDICH,  
OF EDGEWATER PARK, NEW JERSEY.

## MANUFACTURE OF ARTIFICIAL SILK FROM VISCOSE.

No Drawing.

Application filed May 23, 1925. Serial No. 32,454.

My invention relates to the manufacture of filaments by projecting viscose (variously known as cellulose sulphocarbonate or cellulose thiocarbonate) through minute spinneret orifices into baths containing chemicals which coagulate the viscose as a semi-solid impure cellulose hydrate, which must be subjected to subsequent cleaning processes and thereafter dried to form the commercial artificial silk.

Natural silk filaments have an average diameter of .015 millimeter and, therefore, it is highly desirable to produce artificial silk filaments of approximately the same diameter. However, the aforesaid coagulated viscose elements must, of course, be of sufficient strength to withstand the stresses of manipulation incident to their production, and as the viscose products of ordinary processes are much weaker and more frangible than the natural silk filaments; it has been found impossible to commercially manufacture viscose silk filaments which are less than double the diameter of the natural silk filaments. For instance, if dried in air, the minimum diameter of ordinary viscose silk filaments is .03051 millimeter and if viscose silk filaments are subjected to the action of glycerine, as is usual to improve their flexibility, the minimum ultimate diameter attainable is .03545 millimeter.

Therefore, an object and effect of my invention is to provide a method and means for commercially producing viscose silk filaments as fine, lustrous and elastic as natural silk filaments.

Various chemicals are used in the precipitating bath aforesaid. For instance, because of their prompt action and relatively low cost, strong acid baths, such as aqueous solutions containing eight per cent of sulphuric acid or five per cent of hydrochloric acid, are commonly used. With baths of that character, substantially all of the sulphur primarily chemically combined with the cellulose in viscose is released as free sulphur, but is occluded in the mass of cellulose hydrate, causing the latter to present an undesirable dull yellow white appearance, whereas, natural silk has a characteristic lustrous, translucent appearance. Therefore, such ordinary processes of coagulation must be supplemented by successive treatments of the coagulated viscose in chemical baths with a view to removal of the sulphur impurities

therefrom. However, although such cleansing operations are only partially successful, they leave the viscose filaments weak, brittle and inelastic as compared with natural silk.

Microscopic examination of such ordinary viscose silk filaments discloses that their inherent weakness as compared with natural silk filaments is due to the fact that whereas, a natural silk filament is of substantially uniform homogeneous solid structure with a smoothly continuous surface; an ordinary viscose filament is of porous structure with a pitted surface. The formation of such pores and pits is incident to the primary inclusion and occlusion of sulphur derivatives in the cellulose hydrate and subsequent partial elimination of the same, leaving the cellulose hydrate of spongy texture.

Therefore, an object and effect of my invention is to provide a method and means for commercially producing viscose silk filaments without occluding free sulphur or its derivatives therein and to thus strengthen the coagulated cellulose hydrate filament by the elimination of pores and pits as aforesaid, and it is the attainment of that result which permits the formation of filaments, in accordance with this invention, as fine as natural silk filaments.

I have discovered that the desirable results aforesaid are attainable by subjecting viscose to the action of  $\text{PO}_4$  ions. Such ions have a beneficial effect if added to or formed in the viscose, or in any bath in which viscose may be coagulated, or in a fluid distinct from either the viscose or the coagulating medium and, in the latter case, may be either alone or in association with other matter affecting the viscose complex. For instance, the impure cellulose hydrate product of coagulation of viscose may be subjected to  $\text{PO}_4$  ions in a fluid containing dyeing material or detergent material.

$\text{PO}_4$  ions have the apparent effect of preventing the formation of sulphur or its derivatives in insoluble form, and thus render the coagulated products practically self-cleansing. However, if  $\text{PO}_4$  ions be added to or formed in the viscose before coagulating the same in the form of filaments, they have the effect of accelerating the progressive "aging" of the viscose which is manifested by progressive increment in viscosity of the viscose which may or may not be desirable in accordance with the process of coagula-

tion to which the viscose is to be subjected. However, in the form of my invention herein contemplated, I prefer to subject the viscose to the action of  $\text{PO}_4$  ions in a bath in which they are derived from an aqueous solution of tri-sodium phosphate ( $\text{Na}_3\text{PO}_4$ ); although there may be no tri-sodium phosphate present as such in said bath when the viscose is subjected to the action of  $\text{PO}_4$  ions therein.

Although an aqueous solution of either mono-sodium phosphate or di-sodium phosphate, or said tri-sodium phosphate, alone, will effect coagulation of viscose projected therein, particularly if the viscose is of low alkalinity and such solution be hot; I prefer to subject the viscose filament to a preliminary coagulating medium, and such medium may be merely heated atmospheric air.

Therefore my improved process herein claimed may be effected by projecting viscose directly into a heated atmosphere through a spinneret orifice or orifices of such diameter that when subsequently treated and dried the filaments are of the desired degree of fineness; for instance orifices having a diameter of .025 millimeter. Said filaments are thereafter directed from said heated atmosphere into an aqueous solution containing three percent of tri-sodium phosphate ( $\text{Na}_3\text{PO}_4$ ). Such treatment coagulates the viscose to an impure cellulose hydrate complex sufficiently coherent to be mechanically drawn through and from such bath over a roller.

Filaments thus coagulated in accordance with my invention may require no subsequent treatment other than rinsing with water, as they are practically self-cleansing, in such coagulating bath, and emerge therefrom of substantially uniform homogeneous structure and with smooth surfaces. When such filaments are dried, preferably under tension, they have unusually high luster, strength and elasticity, and filaments even finer than natural silk may be thus produced.

Therefore, I do not desire to limit myself to the precise details of structure, arrangement or procedure herein set forth, as it is obvious that various modifications may be made therein without departing from the essential features of my invention, as defined in the appended claims.

However, specific claims for the process of subjecting precipitated viscose to the action of tri-sodium phosphate and for a process in

which viscose is precipitated by any suitable acid before being subjected to the action of tri-sodium phosphate, are included in Letters Patent of the United States 1,576,529 granted to me March 16, 1926 pursuant to application Serial No. 26,825 filed April 29, 1925 and copending herewith.

I claim:

1. The method of manufacturing artificial silk filaments from viscose which consists in coagulating viscose by projecting a fine filament thereof into a coagulating medium and thence into an aqueous solution containing  $\text{PO}_4$  ions.

2. The method of manufacturing artificial silk filaments from viscose which consists in coagulating viscose by projecting a fine filament thereof into a coagulating medium and thence into an aqueous solution containing  $\text{PO}_4$  ions associated with other ions capable of affecting such coagulation.

3. The method of manufacturing artificial silk filaments from viscose which consists in coagulating viscose by projecting a fine filament thereof into a coagulating medium and thence into an aqueous solution containing  $\text{PO}_4$  ions resultant from inclusion of tri-sodium phosphate ( $\text{Na}_3\text{PO}_4$ ) in such solution.

4. The method of manufacturing artificial silk filaments from viscose which consists in coagulating viscose by projecting a fine filament thereof into a coagulating medium and thence into an aqueous solution containing  $\text{PO}_4$  ions, resultant from inclusion of tri-sodium phosphate ( $\text{Na}_3\text{PO}_4$ ) in such solution, with another solute capable of affecting such coagulation.

5. The method of manufacturing artificial silk from viscose which consists in projecting a filament of the latter into a heated atmosphere and thence into an aqueous solution in which tri-sodium phosphate ( $\text{Na}_3\text{PO}_4$ ) has been dissolved.

6. The method of manufacturing artificial silk which consists in projecting a filament of viscose (thiocarbonate) through an orifice less than .025 millimeter in diameter, into the atmosphere, retaining said filament in said atmosphere until partly coagulated, and thence projecting said filament into a bath containing  $\text{PO}_4$  ions.

In testimony whereof, I have hereunto signed my name at Burlington, New Jersey, this 20th day of May, 1925.

WILLIAM MENDEL.